

Patented Jan. 8, 1929.

1,697,907

# UNITED STATES PATENT OFFICE.

HENRY DREYFUS, OF LONDON, AND CLIFFORD IVAN HANEY, OF SPONDON, NEAR DERBY, ENGLAND, ASSIGNEES TO CELANESE CORPORATION OF AMERICA, A CORPORATION OF DELAWARE.

## CELLULOUSIC MATERIAL AND PRODUCT OBTAINED THEREFROM.

No Drawing. Application filed January 19, 1927, Serial No. 162,218, and in Great Britain October 8, 1926.

This invention relates to the treatment of cellulosic materials for the purpose of rendering them more reactive for esterification and especially acetylation and also to the production of cellulose acetates or other cellulose esters from said treated materials.

We have now discovered that cellulosic materials can be rendered more easily esterifiable by treatment with small quantities of formic acid.

The use of small proportions of formic acid is especially valuable in that it is not necessary to subject the cellulosic material to an after treatment for the removal of the formic acid, such as is necessary in the case where larger proportions of formic acid are used. As will be readily understood, in the case where the cellulosic materials are acetylated directly after pretreatment with formic acid, the formic acid in the cellulosic material is destroyed by the acetylating medium used in the subsequent acetylation, the acetic anhydride being simultaneously converted into acetic acid. This by-reaction would occasion a considerable wastage of acetic anhydride where large quantities of formic acid are present, but the loss of acetic anhydride is relatively small when only small quantities of formic acid are present. By the use of small quantities of formic acid in the pretreatment it becomes possible therefore to proceed directly to the esterification of the cellulosic material, without any intermediate treatment for the removal of formic acid by evaporation, or by washing with water followed by a drying operation, or by other methods.

Good results are obtained by the use of 10 to 20 parts by weight of formic acid to each 40 100 parts by weight of cellulosic materials, though the proportions of formic acid used may be greater or less than those indicated. In using very small proportions of formic acid care must be taken to ensure that the 45 cellulosic materials are evenly moistened with the formic acid, while the use of formic acid in proportions exceeding 20 or at most 30% of the cellulosic material only leads to an increase in the wastage of acetic anhydride without any material advantage in other directions.

The formic acid may be employed in a concentrated form or diluted with water

or other diluent. For instance, 100% formic acid, or aqueous solutions containing 50- 55 100% preferably 70-90% formic acid, may be used, or mixtures of formic acid and acetic acid in any desired proportion may also be employed.

As cellulosic materials, we employ cotton, 60 cellulose (in either the mercerized or the non-mercerized form) or wood pulp, the latter having been preferably first submitted to an alkali treatment such as indicated in the British specification No. 249,173 and corresponding U. S. application S. No. 747,054, or other cellulosic materials or their conversion products. The cellulosic material used may contain the usual amount of moisture for example, 4% to 6% or 8%, or may 70 be freed from moisture by drying.

In practising the invention, the formic acid is distributed evenly over the cellulosic material, for instance, by spraying, the cellulosic material being turned or moved from 75 time to time if necessary to ensure uniform impregnation with the formic acid. The cellulosic material is then allowed to stand until a product capable of rapid esterification is obtained.

The time occupied varies with the nature of the cellulosic material, the concentration of the formic acid, the temperature at which the cellulosic material is maintained, and the degree of reactivity required in the product. The treatment proceeds quite satisfactorily at ordinary temperatures but may if desired be accelerated by the use of increased temperatures.

In the subsequent esterification due allowance should be made for the destruction of the esterifying agent by the formic acid present and any water introduced therewith, particularly when working by processes in which minimum quantities of the esterifying medium are used. Thus in acetylation processes, the amount of acetic anhydride is increased by an amount sufficient to convert the water formed by decomposition of the formic acid, together with any water 100 mixed therewith, to acetic acid.

The products may be acetylated with ease and rapidity by any of the usual processes employed for this purpose, provided that the proportion of acetic anhydride is increased 105 in the manner previously indicated, the pro-

portion of acetic acid added being preferably diminished by an amount corresponding with that formed from the excess of acetic anhydride employed.

5 The treatment may be effected in the manner described in the following example, it being understood however, that this example is not to be regarded as limiting the invention in any respect.

10 *Example 1.*

100 parts of cellulose dried or containing for instance 5-6% of moisture, are sprayed with about 15 parts of 75-85% formic acid. 15 The cellulose is allowed to stand until the desired degree of reactivity has been reached, for instance for 8-12 hours, and is afterwards added to an acetylating bath.

20 *Example 2.*

100 parts of cellulose, dried or containing 5-6% of moisture, are moistened with about 20 parts of a mixture containing 30-40% of formic acid and 60-70% of acetic acid. 25 After the desired degree of reactivity has developed, the cellulose is acetylated.

The acetylation may be performed by any suitable process, and especially by the processes described in British specifications Nos. 30 14,101 of 1915, 6,463 of 1915, 100,009, 101,555, corresponding U. S. Patents Nos. 1,278,885, 1,280,974 and 1,280,975, British specification No. 207,562 and corresponding U. S. application S. No. 633,016 filed 18 35 April, 1923, but in the case of cellulose that has been pretreated in accordance with the foregoing example we use about 50 additional parts by weight of acetic anhydride to compensate for the wastage which takes place as the result of the presence of the 40 formic acid in the cellulose.

Thus, to acetylate 100 parts of pretreated cellulose, we may use 900 to 1000 parts by weight of glacial acetic acid, 10 to 15 parts 45 by weight of sulphuric acid and 250 to 300 parts by weight of acetic anhydride.

What we claim and desire to secure by Letters Patent is:—

50 1. A process for treating cellulosic material which comprises treating said cellulosic material with a small proportion of formic acid, thereby producing a cellulose which is highly reactive for esterification.

55 2. A process for treating cellulosic material which comprises treating said cellulosic material with a small proportion of an aqueous solution of formic acid, thereby producing a cellulose which is highly reactive for esterification.

60 3. A process for treating cellulosic material which comprises treating said cellulosic material with a small proportion of formic acid of at least 50% concentration, thereby producing a cellulose which is highly reactive for esterification.

4. A process for treating cellulosic material which comprises treating said cellulosic material with a small proportion of formic acid of at least 70% concentration, thereby producing a cellulose which is highly reactive for esterification. 70

5. A process for treating cellulosic material which comprises treating said cellulosic material with a small proportion of a mixture containing formic and acetic acids, thereby producing a cellulose which is highly reactive for esterification. 75

6. A process for treating cellulosic material which comprises treating said cellulosic material with a small proportion of an aqueous mixture containing formic and acetic acids, thereby producing a cellulose which is highly reactive for esterification. 80

7. A process for treating cellulosic material which comprises treating said cellulosic material with a small proportion of an aqueous mixture containing at least 50% of formic and acetic acids, thereby producing a cellulose which is highly reactive for esterification. 85

8. A process for treating cellulosic material which comprises treating said cellulosic material with a small proportion of an aqueous mixture containing at least 70% of formic and acetic acids, thereby producing a cellulose which is highly reactive for esterification. 90

9. A process for treating cellulosic material which comprises treating said cellulosic material with a proportion not exceeding 30%, calculated on the weight of the cellulosic material, of an aqueous solution of formic acid, thereby producing a cellulose which is highly reactive for esterification. 100

10. A process for treating cellulosic material which comprises treating said cellulosic material with a proportion not exceeding 30%, calculated on the weight of the cellulosic material, of an aqueous solution of formic acid, thereby producing a cellulose which is highly reactive for esterification. 110

11. A process for treating cellulosic material which comprises treating said cellulosic material with a proportion not exceeding 30%, calculated on the weight of the cellulosic material, of a mixture containing formic and acetic acids, thereby producing a cellulose which is highly reactive for esterification. 115

12. A process for treating cellulosic material which comprises treating said cellulosic material with a small proportion of formic acid, thereby producing a cellulose which is highly reactive for esterification, and subjecting the resulting cellulose to the action of an esterifying medium. 120

13. A process for treating cellulosic material which comprises treating said cellu- 125

losic material with a small proportion of an aqueous mixture containing formic acid, thereby producing a cellulose which is highly reactive for esterification, and subjecting 5 the resulting cellulose to the action of an esterifying medium.

14. A process for treating cellulosic material which comprises treating said cellulosic material with a small proportion of a 10 mixture containing formic and acetic acids, thereby producing a cellulose which is highly reactive for esterification, and subjecting the resulting cellulose to the action of an esterifying medium.

15. 15. A process for treating cellulosic material which comprises treating said cellulosic material with a small proportion of formic acid, thereby producing a cellulose which is highly reactive for esterification, 20 and subjecting the resulting cellulose to the action of an esterifying medium for the production of carboxylic acid esters.

16. A process for treating cellulosic material which comprises treating said cellulosic material with a small proportion of formic acid, thereby producing a cellulose which is highly reactive for acetylation, and 25

subjecting the resulting cellulose to the action of an acetylating medium.

17. A process for treating cellulosic ma- 30 terial which comprises treating said cellulosic material with a proportion not exceeding 30%, calculated on the weight of the cellulosic material, of an activating agent comprising formic acid, thereby producing 35 a cellulose which is highly reactive for acetylation, and subjecting the resulting cel- lulose to the action of an acetylating me- dium.

18. A process for treating cellulosic ma- 40 terial which comprises treating said cellulosic material with a proportion not exceeding 30%, calculated on the weight of the cellulosic material, of an activating agent comprising formic and acetic acids, thereby 45 producing a cellulose which is highly re- active for acetylation, and subjecting the resulting cellulose to the action of an acetyl- ating medium.

In testimony whereof we have hereunto 50 subscribed our names.

HENRY DREYFUS.  
CLIFFORD IVAN HANEY.